

## UNITED STATES PATENT OFFICE.

CHARLES S. HOLLANDER, OF PHILADELPHIA, PENNSYLVANIA, ASSIGNOR TO  
ROHM & HAAS COMPANY, A CORPORATION OF DELAWARE.

USE OF HYDROSULPHITES OR SULFOXYLATES IN THE REMOVAL OF DYES FROM  
TEXTILE FIBERS.

No Drawing.

Application filed June 9, 1925. Serial No. 36,022.

For some time it has been known that dyes can be stripped from textile fabrics by the use of basic zinc sulfoxylate formaldehyde. However, since this material is only very sparingly soluble in water, it has always been used in the presence of either an acid or an alkali, either of which would cause it to dissolve rapidly. However, acids have a very injurious action on vegetable fibers, whereas, alkalis damage animal fibers. Accordingly, this material has not been considered as being readily available for stripping dyes from mixed fabrics.

I have now found that basic zinc sulfoxylate formaldehyde can be used as a stripping agent in the presence of a salt such as sodium chloride, sodium sulphate, sodium acetate, potassium chloride, potassium sulphate, ammonium chloride or ammonium sulphate as well as many others. These salts (all of which include as a base a substance whose hydroxide is strongly alkaline), while they may show some acid or alkaline reaction to litmus, are substantially neutral in effect as regards the injury to either animal or vegetable fibers. I therefore classify them broadly under the term "substantially neutral salts of substances whose hydroxides are strongly alkaline." It may be noted that all of these salts are readily soluble in water. When such a neutral salt is used the basic zinc sulfoxylate formaldehyde does not go quickly into solution as is the case when an acid or an alkali is used, but nevertheless does accomplish the desired result. Basic zinc sulfoxylate formaldehyde is ordinarily classed as an insoluble substance. However, in hot water it will form a slight solution (of approximately 1% strength), and this is sufficient to cause the foregoing reaction to take place. Despite the fact that this material is thus slightly soluble, it may properly be termed "a substantially insoluble sulfoxylate formaldehyde." An explanation of this would be that in water solution, especially



The water soluble ammonium sulfoxylate formaldehyde in this case accomplishes the stripping and as the dyes are stripped, this material is consumed. This in turn upsets the equilibrium and more ammonium sulfoxylate formaldehyde is formed until the desired result is accomplished.

The following are given as examples of my process, but it is to be understood that they are given only by way of illustration and I do not intend to limit myself as to the time, temperature, percentages, proportions or sequence of operations:

*First example.*—100 parts of dyed goods composed of wool and cotton were heated with enough water to completely immerse them. 10% of a mixture of equal parts of basic zinc sulfoxylate formaldehyde and of ammonium chloride were added and stirred in. The goods were then heated at a temperature of 180° F. to 212° F., until the color had been discharged. They were then rinsed thoroughly with water and dried in the usual manner.

*Second example.*—100 parts of a mixture of silk and cotton fibers may be discharged by immersing them in water, bringing to boil and adding 5% of basic zinc sulfoxylate formaldehyde and 5 to 10% of ordinary table salt. The boiling should continue until all the dye has been discharged then thoroughly rinsed and dried in the usual manner.

It may be found necessary to prepare the goods for the stripping action by removing the adhering dirt and grease with a weak soap solution or any other means usually employed by the trade for this purpose.

What I claim is:—

1. Process of stripping dyes from dyed materials which consists in immersing such materials in a mixture of a substantially insoluble sulfoxylate formaldehyde and a readily soluble substantially neutral salt of a substance whose hydroxide is strongly alkaline.
2. A process as defined in claim 1, in which the solution is heated to approximate-

ly the boiling point during the stripping operation.

3. A composition of matter adapted for use in stripping dyes from textile fabrics and the like, comprising a mixture of substantially insoluble sulfoxylate formaldehyde and a readily soluble, substantially neutral salt of a substance whose hydroxide is strongly alkaline.

CHAS. S. HOLLANDER.